

April 19, 1949.

W. R. PRATT

2,467,596

MANUFACTURE OF ABRASIVE WHEELS

Filed Nov. 8, 1946



*Fig. 1.*

17 19 12

*Fig. 2.*



*Fig. 3.*



WILLARD R. PRATT  
INVENTOR.

BY *Malvin White*

ATTORNEY

## UNITED STATES PATENT OFFICE

2,467,596

## MANUFACTURE OF ABRASIVE WHEELS

Willard R. Pratt, Los Angeles, Calif., assignor to  
 Bevil Company, San Francisco, Calif., a co-partnership

Application November 8, 1946, Serial No. 708,613

6 Claims. (Cl. 51—293)

1

This invention has to do with improved methods for the manufacture of abrasive wheels of the general form embodying a metallic center or core carrying an abrasive rim. Particularly the invention is concerned with considerations having to do with the bonding of the rim to the core, and where the rim may be composed of pre-formed individual segments, with the inter bonding of those segments to form an integrated rim annulus.

At the outset it may be observed that the invention deals with abrasive wheels having sintered rims, by which I mean rim compositions formed for example of pulverulent metal containing uniformly distributed diamond particles, integrated by heating to a temperature of incipient fusion or sintering of metallic particles, and at which the composition at all times remains essentially solid, though perhaps slightly plastic at the maximum temperature to which it is subjected.

Considering first the problem of bond formation between the core and the heated essentially solid rim, my primary concern is to create a fusion formed bond while exteriorly confining the rim and expanding the core into tight or even penetrating engagement with the rim. Difficulties have arisen however because of the fact that upon expansion of the core, the rim material is bodily displaced or expanded against the confining medium or mold with such force as not infrequently to rupture the mold.

The invention affords a solution of the difficulty by permitting an expansion range for both the core and rim within an initial and considerable expansion range, and final confinement against further expansion of the rim at a point in such relation to the temperature rise that the core to rim bond formation will occur while the rim is strongly pressed between the core and mold, but without the latter being subjected to breaking pressure. The considerations thus taken into account for the bonding of sintered rims to their cores has given rise to advantages and facilities unattainable by any of the various practices heretofore used or proposed for abrasive wheel manufacture.

In accordance with the invention, the core and rim are placed in a mold, the material of which is specially regarded as to its co-efficient of expansion relative to the expansion properties of the core. Preferably I use a graphite mold, because of the low coefficient of expansion of graphite, of sufficient, but not necessarily of excessive wall thickness, to withstand the highest pressure to be transmitted by the rim. The rim

2

material is placed in the mold about the core in such relation that the rim material occupies less than the radial distance between the mold wall and core. Thus clearance space initially may exist beyond either or both the inner and outer edges of the rim.

Thereafter, as the assembly is heated, the resultant expansion of the core, or core and rim, is accommodated throughout an initial range in taking up, so to speak, the clearance space or spaces. In the course of the expansion, the solid rim is radially displaced or compressed, ultimately to a point of pressing strongly against the circular mold wall because of the pressure transmitting qualities of the sintered rim material. However, since such pressure exertion against the mold occurs only toward the end of the expansion range, such pressure will not assume a rupturing magnitude.

Since dimensional relationships are of significance, it may be preferred to first sinter the rim material before placing it in the mold for bonding to the core, with the advantage that having been compacted and presintered, the rim will have reached more accurately predetermined and stable physical and dimensional characteristics.

It is contemplated that the rim may be composed of preformed segments to be placed in an annular arrangement about the core. The aforementioned advantages obtain in this instance, with the further effects of the core expansion to displace or crowd the segments toward their interengagement, and resultant tight pressure of one against the other as where the segments are themselves to be bonded together.

Other features and objects of the invention are directed to the maintenance or placement in the interfaces between either or both the core and rim, and between rim segments, of a relatively low melting temperature metal which is subjected to compression by the expansion forces of the core and rim, and which melts to form an alloy bond between the interface surfaces.

More complete understanding of the invention will be had from the following detailed description throughout which reference is had to the accompanying drawing, in which:

Fig. 1 is a sectional view showing the core and abrasive rim within a typical form of mold assembly;

Fig. 2 is a cross-section on line 2—2 of Fig. 1; and

Fig. 3 is a view similar to Fig. 2 illustrating a variational procedure contemplated by the invention.

It is contemplated that the abrasive rim initially and before bondage to the core, may be formed as a complete annulus, or as segments to be placed in the mold in annular arrangement about the core. Fig. 2 shows the rim 10 to consist of a preformed annular compact, composed typically of finely divided nickel (passing a 325 mesh screen) containing a uniform distribution of small diamond particles. The compact initially will have been formed under high pressure to assume a self-sustaining shape, and desirably may have been heated to sintering temperature, resulting in a preformed annulus having, by reason of its sintered condition, the advantages of more accurate predetermination of its dimension and other physical characteristics.

The rim 10 is placed in a mold assembly 11 about a core 12, typically in the form of a circular steel disc whose thickness is less than the rim thickness. The mold assembly comprises a pair of identical mating sections 13 and 14, the latter of which has a cylindrical bore 15 receiving the corresponding size lower portion 18a of the section above. The rim 10 is received within opposed annular recesses 16 within the end faces of the mold sections, while the core 12 is flatly engaged between the mold surfaces 17 surrounded by the recesses. One mold section may carry an axial projection 18 receivable through opening 19 in the disc within bore 20 of the companion section, to accurately center the core with relation to mold wall surface 15.

As previously explained, the rim 10 is preformed to occupy, when first placed in the mold, a space less than the radial distance between the rim of the core 12 and the mold wall 15. Thus as shown in Fig. 2, the rim may have clearances at either or both 21 and 22, respectively between the rim and core, and between the rim and mold wall. The amount of clearance in any given instance will depend upon such considerations as the diameter of the wheel and the expansion characteristics of the core, or the differential expansion, upon heating, of the core and mold. Using a graphite mold, having relatively low coefficient of expansion, the tendency upon heating the assembly will be for the steel core to expand and ultimately close such clearance spaces as will initially have existed at either or both the inside and outside of the rim.

With the rim and core placed in the mold in the condition illustrated by Figs. 1 and 2, the mold assembly is placed in a furnace and heated to a temperature which will not exceed the sintering temperature of the rim composition, and will therefore permit the rim to at all times remain an initially solid mass. Pressure may or may not be applied to the rim and disc during the heating. Pressure, if desired, may be applied in any suitable manner, as by means of plunger 23 bearing against the upper mold section. As the heating and temperature rise progress, the core 17 expands, together with some expansion of the rim 10, to completely close the clearance spaces at 21 and 22, this condition preferably being reached as the maximum temperature is approached, so that subsequent expansion will bring the core into tightly pressed engagement with the rim, and the rim into tightly pressed engagement with the mold surface 15, but without the exertion of such excessive pressure as will rupture the mold. Preferably the parts will be so dimensionally related that at the highest temperature and point of maximum expansion, the core will have slightly penetrated the rim ma-

terial, the latter having at its sintering temperature sufficient plasticity to permit its penetration by the core, but without having the free mobility of a fluid.

For purposes of the bond formation between the core and rim, provision is made for making available at the core-rim interface a metal whose melting temperature is low with relation to the melting point of the rim matrix metal, in this case typically nickel, so that at the rim sintering temperature, the interface metal will melt and form a bonding alloy solution with the core and rim metals. Best results are obtained using the low melting temperature metal in a very thin form, as for example by electroplating on the rim surface of the core, or by applying to either the rim or core surfaces at the interface a thin coating of the metal, or by insertion of a thin foil of the metal between the interface surfaces. Excellent bonds have been obtained by inserting within the interface space a foil of copper, or copper-containing alloy, the thickness of the foil being not in excess of about 0.002 inch. Upon heating, the foil melts and goes into alloy solution with the interface metals at a relatively low temperature, within the range of from 1500° F. to 2000° F., thus enabling the bond to be formed at such low temperatures and without having to reach the relatively high temperatures required for alloy formation at the interface in the absence of the low melting temperature metal. Upon examination of the resulting bond, the copper or copper alloy, will be found to have virtually disappeared by having gone into alloy solution. Of course the effectiveness of the bond formation is further increased by the fact that the core expansion will have kept the foil under tight compression between the core and remain as the copper melts and alloys with the interface metals.

Fig. 3 illustrates the adaptation of the invention for bonding to the rim a preformed segmental rim. Here the rim 25 is shown to be composed of segments 26 preformed as self-sustaining compacts, which as in the case of the first described rim 10, may initially have been sintered. The segments are placed in the mold about the core 27 with clearances at 28 or 29, or both, respectively at the inside and outside of the segments. The arcuate dimensions of the latter may be such that the end surfaces at 30 of adjacent segments may initially be in close proximity or ultimately brought into pressed inter-engagement upon expansion of the core and by virtue of the degree of mobility which the compacts have at sintering temperature.

As before, relatively low temperature melting metal, e. g. copper foil, is inserted within the interface at 28, and where bonds are to be formed between the segments themselves, the foil may be inserted also within the interfaces at 30. Upon heating of the assembly to the compact sintering temperature, the low melting temperature metal results in alloy bond formations between the segments and core, and between the segments themselves where the low melting temperature metal is placed within the interfaces 30 for this purpose. As will be understood, the relationship between the clearance spaces and core expansion, and eventual pressed radial confinement of the rim between the core and the mold wall, are essentially the same as in the first described instance.

I claim:

1. The method of making abrasive wheels that

includes, placing a metallic core within and in annularly spaced relation to the wall of a mold, placing between said core and wall a relatively high melting temperature rim compact composed of abrasive particles and matrix metal and occupying less than the radial distance between said core and wall, heating the mold, core and rim to a temperature below the melting temperature of the compact and at which the compact remains an essentially solid mass to resist expansion of the core, producing by said heating radial expansion of the core into tight engagement with the solid rim and resultant strongly pressed engagement of the rim against said mold wall, and simultaneously forming a fused bond between said core and rim in the presence of a relatively low melting temperature metal between said core and rim.

2. The method of making abrasive wheels that includes, placing a metallic core within and in annularly spaced relation to the wall of a mold, placing between said core and wall a relatively high melting temperature rim compact composed of abrasive particles and matrix metal and comprising a plurality of individual segments occupying less than the radial distance between said core and wall, heating the mold, core and rim to a temperature below the melting temperature of the compact and at which the compact remains an essentially solid mass to resist expansion of the core, producing by said heating radial expansion of the core into tight engagement with the solid rim and resultant strongly pressed engagement of the rim against said mold wall, and simultaneously bonding said segments together and to said core in the presence of a relatively low melting temperature metal tightly pressed by said core expansion between the segments and core and which forms an alloy with the core.

3. The method of making abrasive wheels that includes, placing a metallic core within and in annularly spaced relation to the wall of a mold, placing between said core and wall a rim compact composed of abrasive particles and matrix metal and occupying less than the radial distance between said core and wall, maintaining between the core and rim a relatively low melting temperature metal, heating the mold, core and rim to a temperature below the melting temperature of the compact and at which the compact remains an essentially solid mass to resist expansion of the core, producing by said heating radial expansion of the core to tightly press said low melting temperature metal between the core and rim and to strongly press the rim against said mold wall, and simultaneously melting said low melting temperature metal to form at the interface between said core and rim a bond composed of alloy of said low melting temperature metal and the core and rim metals.

4. The method of making abrasive wheels that includes, placing a metallic core within and in annularly spaced relation to the wall of a mold, placing between said core and wall a rim compact composed of abrasive particles and matrix metal and occupying less than the radial distance between said core and wall, maintaining between the core and rim a foil-like layer of relatively low melting temperature metal, heating the mold, core and rim to a temperature below the melting temperature of the compact and at which the compact remains an essentially solid mass to resist expansion of the core, producing by said heating radial expansion of the core to tightly press said low melting temperature metal be-

tween the core and rim and to strongly press the rim against said mold wall, and simultaneously melting said low melting temperature metal to form at the interface between said core and rim a bond composed of alloy of said low melting temperature metal and the core and rim metals.

5. The method of making abrasive wheels that includes, placing a metallic core within and in annularly spaced relation to the wall of a mold, placing between said core and wall a rim compact composed of abrasive particles and matrix metal and comprising a plurality of individual segments occupying less than the radial distance between said core and wall, maintaining between said segments and between the segments and rim a relatively low melting temperature metal, heating the mold, core and rim to a temperature below the melting temperature of the compact and at which the compact remains an essentially solid mass to resist expansion of the core, producing radial expansion of the core to tightly press said low melting temperature metal between the core and rim and to strongly press the rim against said mold wall, and simultaneously melting said low melting temperature metal to form at the interfaces between the segments and between the core and segments bonds composed of alloy of said low melting temperature metal and the core and rim metals.

6. The method of making abrasive wheels that includes placing a metallic core within and in annularly spaced relation to the wall of a mold, placing between said core and wall a rim compact composed of abrasive particles and matrix metal and comprising a plurality of individual segments occupying less than the radial distance between said core and wall, placing between the segments and between the segments and rim relatively low melting temperature metal foil, heating the mold, core and rim to a temperature below the melting temperature of the compact and at which the compact remains an essentially solid mass to resist expansion of the core, producing by said heating radial expansion of the core to tightly press said low melting temperature metal between the core and rim and to strongly press the rim against said mold wall, and simultaneously melting said foil to form at the interfaces between the segments and between the core and segments bonds composed of alloy of said low melting temperature metal and the core and rim metals.

WILLARD R. PRATT.

#### REFERENCES CITED

The following references are of record in the file of this patent:

#### UNITED STATES PATENTS

| 60         | Number          | Name           | Date |
|------------|-----------------|----------------|------|
| Re. 21,165 | Van der Pyl     | July 25, 1939  |      |
| 1,833,099  | Welch           | Nov. 24, 1931  |      |
| 1,848,182  | Koebel          | Mar. 8, 1932   |      |
| 2,019,934  | Schroter et al. | Nov. 5, 1935   |      |
| 2,173,835  | Boyer et al.    | Sept. 26, 1939 |      |
| 2,189,259  | Van der Pyl     | Feb. 6, 1940   |      |
| 2,405,086  | Bevillard       | July 30, 1946  |      |

#### OTHER REFERENCES

"Best Joint Designs for Silver Alloy Brazing," F. T. Van Syckel, The Welding Journal, August, 1941, pages 527 and 529.

"Tool Tipping Data," The Welding Journal, July, 1943, page 61, Engineering Data Sheet No. 75 24.